

# UNITED STATES PATENT OFFICE.

WILLIAM AUGUSTUS HALL, OF NEW YORK, N. Y.

## ART OF COLORING WOOD.

No. 901,098.

Specification of Letters Patent.

Patented Oct. 13, 1908.

Application filed February 1, 1908. Serial No. 413,762.

*To all whom it may concern:*

Be it known that I, WILLIAM AUGUSTUS HALL, a citizen of the United States, residing at New York, in the county of New York and State of New York, have invented or discovered certain new and useful Improvements in the Art of Coloring Wood, of which the following is a specification.

This invention relates to the art of coloring wood so as to produce from some of the cheaper or more common varieties of hard-wood, such as birch, beech, or maple, close imitations of rarer or more expensive woods, such as mahogany or walnut; and the invention has for its object to color the wood throughout to uniform shades, so that when cut up in making cabinet work, or for other purposes, there will be no streaked or uncolored parts, and the close imitations of more expensive woods will therefore be preserved.

In the coloring of hardwoods by the vacuum and pressure process it has been found, in the treatment of lumber containing both the sap and heart of wood (and which is about the only kind commercially obtainable) that a desired uniform coloring is not produced, for the reason that the coloring solution saturates the more porous portions, which is the sap wood, and such portions of the heart wood as are weak structurally, but is not diffused or uniformly distributed throughout the denser parts of the wood. In almost every case wood thus treated, even for the longest time, and under the highest pressure practicable, will show totally uncolored or very slightly colored streaks or patches which render the same undesirable for commercial utilization. It has been discovered that this streaky effect can be overcome only by a diffusion of the color throughout the wood and that this can best be effected by a slow cooking or boiling for a considerable time and at relatively low temperature. It is, however, impracticable to do this in the cylinders in which the wood has been treated, for the reason that the diffusion requires several days, and as the cylinder apparatus is very expensive it is not economical to utilize it for this purpose. Furthermore, the diffusion must be effected without any pressure and at a temperature not to exceed 212° F., so that the wood will not be injured by being subjected for a long time to high temperatures.

In practicing the invention well-seasoned

lumber is put into a cylinder or other suitable chamber and is then preferably heated by indirect steam or otherwise to about 225° F. A vacuum of about twenty-five inches is then applied to withdraw the air from the cells of the wood, the previous heating of the wood facilitating the removal of the air. After the air is completely removed a coloring solution, such as may be made from bark extracts or anhydrides of tannin, or from any suitable stains or dyes, is admitted to the chamber of the cylinder and is forced into the wood, under pressure. The pressure is maintained from six or eight hours to fifteen or twenty hours, according to the hardness and thickness of the wood, and the latter is then removed from the cylinder, and if examined internally will be found to present a streaky and partially colored appearance. The lumber is then preferably placed in open vats in which it is slowly boiled or cooked preferably in the same solution with which it was treated in the cylinder, or in a similar solution, and for a period of several days. If, however, the boiling be done in a closed receptacle it should be done at atmospheric pressure, so that the temperature will not exceed 212° F. This slow boiling or cooking causes a general diffusion of the color in the wood so that it will be of a uniform shade throughout.

Thick lumber is difficult to color in an open vat, for the reason that the air in the cells in the central or inner parts of the wood acts as a repelling cushion, preventing proper circulation or penetration of the coloring solution, so that, in such case, when the lumber is removed from the coloring solution the wood has an uncolored inner portion or core. But by removing this air cushion by the vacuum process it becomes possible to cause the coloring solution to penetrate into the central parts of the wood, although this penetration is not uniform, and the coloring solution will be lodged largely in the ducts or pockets in the more porous portions and concentric rings, and it cannot be uniformly distributed throughout by any amount of pressure which may be applied. This uniform distribution or diffusion of the coloring matter which has thus been forced into the wood can, however, be effected by cooking or boiling the wood for a long time at relatively low temperatures and preferably in an open vat, as hereinbefore described; and this cooking or boiling in the coloring solution at rel-

atively low temperatures is found to be more effective for a uniform diffusion of the coloring material throughout the wood than a hard boiling at high temperatures and under high pressure, and also avoids injuring the strength of the lumber which is likely to occur where the wood is subjected to high temperatures for any considerable length of time.

10 Having thus described my invention or discovery I claim and desire to secure by Letters Patent:—

1. The herein-described process for coloring wood, consisting in subjecting well-seasoned lumber to the action of a vacuum in a closed chamber or receptacle, to draw the air therefrom and render the same absorbent, then forcing a coloring solution into and throughout the wood, so far as practicable, by high pressure, and subsequently diffusing the coloring matter in the wood by boiling or cooking the latter for a long time in the coloring solution at a temperature not exceeding 212° F.

25 2. The herein-described process for coloring wood, consisting in heating well-seasoned lumber in a closed chamber or receptacle, then subjecting the same to the action of a vacuum, to draw the air therefrom and render the wood absorbent, then forcing a coloring solution into and throughout the wood, so far as practicable, by high pressure, and subsequently diffusing the coloring matter in

the wood by boiling or cooking the latter for a long time in the coloring solution at a temperature not exceeding 212° F. 35

3. The herein-described process for coloring wood, consisting in subjecting well-seasoned lumber to the action of a vacuum in a closed chamber or receptacle, to draw the air therefrom and render the same absorbent, then forcing a coloring solution into and throughout the wood, so far as practicable, by high pressure, and subsequently diffusing the coloring matter in the wood by boiling or 40 cooking the latter for a long time in the coloring solution in an open vat or receptacle. 45

4. The herein-described process for coloring wood, consisting in heating well-seasoned lumber in a closed chamber or receptacle, 50 then subjecting the same to the action of a vacuum, to draw the air therefrom and render the wood absorbent, then forcing a coloring solution into and throughout the wood, so far as practicable, by high pressure, and 55 subsequently diffusing the coloring matter in the wood by boiling or cooking the latter for a long time in the coloring solution in an open vat or receptacle.

In testimony whereof I affix my signature, in presence of two witnesses.

WILLIAM AUGUSTUS HALL.

Witnesses:

ANNIE B. WALTERS,  
C. M. SWEENEY.